

## UNITED STATES PATENT OFFICE

2,198,762

## MAGNESIUM ALLOY

Fritz Christen, Zurich-Altstetten, Switzerland

No Drawing. Application May 31, 1939, Serial  
No. 276,716. In Switzerland September 16,  
1938

3 Claims. (Cl. 75—168)

The invention relates to the production of magnesium alloys.

The magnesium alloys hitherto known for casting in sand and metal moulds do not exhibit sufficient tensile strength even if they are subjected to improvement, viz. quick cooling followed by re-heating, and they also exhibit defects in respect of adequate ductility so that the possibility of using them is still very limited.

The object of the present invention is to provide an improved magnesium alloy in which these defects do not appear.

According to the present invention this object is attained by an alloy of magnesium with from 3 to 12% of the pre-alloy or master-batch alloy according to co-pending application Serial No. 243,657, which pre-alloy consists of:

|           | Per cent |
|-----------|----------|
| Aluminium | 43.5-41  |
| Zinc      | 26-30    |
| Manganese | 1.5-3    |
| Nickel    | 3-6      |
| Steel     | 5-2      |
| Magnesium | 21-18    |

The alloy according to the invention thus has a composition falling within the following limits:

|           | Per cent    |
|-----------|-------------|
| Aluminium | 1.23-5.22   |
| Zinc      | 0.78-3.6    |
| Manganese | 0.045-0.36  |
| Nickel    | 0.09-0.72   |
| Steel     | 0.06-0.60   |
| Magnesium | 90.16-97.63 |

For producing an alloy within the foregoing range which after being cast in sand moulds exhibits high tensile strength and high ductility, the composition may be as follows:

|           | Per cent |
|-----------|----------|
| Aluminium | 4        |
| Zinc      | 3        |
| Manganese | 0.1      |
| Nickel    | 0.2      |
| Steel     | 0.2      |
| Magnesium | 92.5     |

An alloy which has high ductility in association with moderate tensile strength has the following composition:

|           | Per cent |
|-----------|----------|
| Aluminium | 2        |
| Zinc      | 3.5      |
| Manganese | 0.3      |
| Nickel    | 0.5      |
| Steel     | 0.1      |
| Magnesium | 93.6     |

In all cases, the alloys are produced in the following way. First of all an alloy as prescribed in co-pending application Serial No. 243,657 is produced with the requisite quantities of aluminium, zinc, manganese, nickel and steel, and the appropriate amount of magnesium as specified in the said application. Pigs of this pre-alloy are placed in the furnace and are covered with a covering salt of known composition which comprises magnesium chloride. When the material has liquefied, pig magnesium is added to the requisite amount and a fresh covering of salt is applied. After a temperature of about 950° C. has been reached heating is discontinued and the liquid metal which is somewhat superheated is thoroughly stirred and is covered again. After the temperature has dropped to about 800° C. the slag is removed and the alloy is cast in moulds of the desired dimensions at about 700° C.

I claim:

1. As an article of new manufacture, a magnesium alloy having a composition falling within the range:

|           | Per cent    |
|-----------|-------------|
| Aluminium | 1.23-5.22   |
| Zinc      | 0.78-3.6    |
| Manganese | 0.045-0.36  |
| Nickel    | 0.09-0.72   |
| Steel     | 0.06-0.60   |
| Magnesium | 90.16-97.63 |

2. As an article of new manufacture, an alloy consisting of:

|           | Per cent |
|-----------|----------|
| Aluminium | 4        |
| Zinc      | 3        |
| Manganese | 0.1      |
| Nickel    | 0.2      |
| Steel     | 0.2      |
| Magnesium | 92.5     |

3. As an article of new manufacture, an alloy consisting of:

|           | Per cent |
|-----------|----------|
| Aluminium | 2        |
| Zinc      | 3.5      |
| Manganese | 0.3      |
| Nickel    | 0.5      |
| Steel     | 0.1      |
| Magnesium | 93.6     |

FRITZ CHRISTEN.